

May 22, 1928.

1,671,022

A. C. FISCHER

PREFORMED RAIL FILLER

Filed June 30, 1927



Inventor:  
Albert C. Fischer,

By Ballard Moreau attorney

## UNITED STATES PATENT OFFICE.

ALBERT C. FISCHER, OF CHICAGO, ILLINOIS.

## PREFORMED RAIL FILLER.

Application filed June 30, 1927. Serial No. 202,580.

My invention relates to a preformed rail filler comprising a prepared strip of waterproofing material, preferably bituminous material, or other suitable binder shaped to conform to the outline of the rail on one side and suitably faced for contact with the paving on the other side, the strip being adapted to act as an insulating, sound deadening and expansion material, deadening the sound of the car upon the rail and insulating the track from the adjacent paving material, and taking up expansion and contraction between them.

My invention is concerned more with the substance out of which the strips are made rather than to their particular form.

One of the objects of my invention resides in providing a preformed rail filler comprising waterproofing binder and granulated cork, suitably intermixed, not only to assist in the insulating and sound deadening characteristics of the strip, and providing an efficient flow retarder for the compressible waterproofing binder, such as bituminous material, but also providing expansibility and compressibility of the strip.

These and other objects of my invention will be apparent from a perusal of the following specification when taken in connection with the accompanying drawings, wherein,

Figures 1 to 6 inclusive illustrate various designs of strips which may be used singly or collectively in connection with the rail filler, after the manner illustrated and claimed in an application filed by H. W. Herbst on January 6, 1926, Serial No. 79,543.

It is understood that any of the blocks or strips shown in my joint application aforesaid, or any other type of strip may be availed of, the present invention being concerned with the material of which the rail filler strips are composed.

The present application contains subject matter withdrawn from the application Serial No. 79,543, the former case being limited to the shape and construction of the rail filler, and the present case being limited to the materials used in making the rail filler.

In my present invention I propose to form my rail filler of a mixture of waterproofing material and a cellular, granular filler, the same preferably being granulated cork, al-

though the invention is not restricted thereto, but broadly comprehends material of any granular form.

As an alternative construction I may, however, if desired, add to the cork finely divided fibrous material, or I may add linear fibres, the latter of which gives strengthening characteristics to the rail filler, while the former merely acts as a flow retarder and lends compressibility to the strip.

The waterproofing binder may consist of a suitable blown asphalt or any other suitable bituminous material having binding and waterproofing qualities.

The waterproof binder as a modified form may consist of bituminous material having added thereto dissolved rubber, or resin.

The proportion of granulated cork may run as high as twenty-five per cent, or more, but preferably twenty-five per cent mixed with approximately seventy-five per cent of the bituminous material.

The binder may be suitably mixed with the granulated cork and/or the linear fibres in a suitable power mixer, and extruded, rolled, molded or pressed into form.

In certain instances I may also add to any of the substances above noted, or any combination of them, earthy or mineral material, since it facilitates the extrusion and provides a cheap filler. These earthy materials may include limestone dust, slate particles, infusorial earth, clay and others, and may be used in amounts from ten to twenty per cent.

It can readily be understood that the incorporation of the cork granules either with or without linear fibrous material in the bituminous material will insulate the granite, concrete or brick paving about the rail, and the compressible and cellular structure of the granules will take up the sound and prevent its transmission from the rail to the hard paving substance.

The binder with the aid of the filler will also provide a suitable expansion joint material, due to the compressible qualities of the bituminous or like material, and the resiliency of the cork granules and/or the linear fibres. These elements serve to take up vibration.

I claim:

1. A preformed rail filler adapted for use as an insulator, sound deadener and expansion joint, comprising a homogeneous mix-

ture of waterproof binder and granulated cork.

2. A preformed rail filler adapted for use as an insulator, sound deadener and expansion joint, comprising a homogeneous mixture of waterproof material, granulated cork and linear fibres.

3. A preformed rail filler adapted for use as an insulator, sound deadener and expansion joint, comprising a homogeneous mixture of waterproof binder, granulated cork, finely divided fibres and an earthy material.

4. A preformed rail filler adapted for use

as an insulator, sound deadener and expansion joint, comprising a homogeneous mixture of waterproof binder and compressible granular materials.

5. A preformed rail filler adapted for use as an insulator, sound deadener and expansion joint, comprising a homogeneous mixture of waterproof material, compressible granular material, and linear fibers.

Signed at Chicago, Illinois, this 16th day of June 1927.

ALBERT C. FISCHER.